

## UNITED STATES PATENT OFFICE

2,089,034

## METHOD OF MAKING LAMINATED PRODUCTS

James V. Nevin, Aberdeen, Wash.

No Drawing. Application August 12, 1935.  
Serial No. 35,885

3 Claims. (Cl. 144—309)

This invention relates to a method of making laminated products, and more particularly to a method of making plywood using a fibrous web impregnated with an aqueous resin-forming binding agent to effect a bond between the constituent laminations of the plywood.

It has heretofore been proposed to impregnate fabrics and the like with solutions of a synthetic resin of the phenol-aldehyde type in an organic solvent, but in addition to the higher cost of such solutions, difficulties are experienced in their use due to the penetrative ability of the solutions. The organic solvents ordinarily employed penetrate deeply into the veneers, often forming pockets which are sources of trouble in the hot pressing operation owing to the fact that great vapor pressures are frequently developed in them that prevent the veneers from making proper contact. Such vapor pressure pockets occasionally result in the explosion of the panel when removed from the press and generally cause defective bonding between the laminations.

I have now found that if the resin forming binding agent is made up into an aqueous solution and the fibrous web impregnated therewith, the cost of manufacture is greatly reduced and the difficulties due to the formation of vapor pressure pockets is largely eliminated. I have also found that a firmer and more satisfactory bond is obtained if the impregnated web is humidified to a substantial moisture content before being interposed between the other laminations and inserted in the hot presses. The layer or film carrying the binding agent may also be used as a surface coating for the faces of either plywood or fiber board panels when a smooth surface is desired.

It is therefore an important object of this invention to provide a method for making laminated products wherein a carrier film or web impregnated with an aqueous solution of a binding agent is employed as the bonding medium for wood veneers or wood fiber board, or as a surface layer therefor.

It is also an important object of this invention to provide a method for the manufacture of plywood and the like which includes the use of a carrier film or web impregnated with an aqueous solution of a resin-forming binding agent and wherein the impregnated carrier film is humidified prior to the hot pressing operation and the product coming from the hot presses is again humidified to give a finished product that will stand up under all climatic conditions.

Other and further important objects will be

come apparent from the following description and appended claims.

The carrier film or web that I impregnate with an aqueous solution of a resin-forming binding agent may be any suitable porous, flexible, fibrous sheet material, such as a fabric or an unsized paper. Unsized kraft paper or toweling has been found to be particularly suitable, since it has sufficient wet strength to withstand the slight tension to which it is subjected after it has been saturated with the aqueous binder solution. The paper may be either bleached or unbleached.

In order to impregnate the carrier film or web, it is conducted through a set of pressure rolls, one or both of which are immersed in a very viscous aqueous solution of the resin-forming binding agent. As the carrier film passes between the pressure rolls, the aqueous solution of the binding agent is forced directly into the absorbent film. The viscosity of the aqueous solution of the binding agent can be adjusted so as to give either a light or heavy coating or impregnation, as desired.

After impregnation of the carrier film or web with the aqueous solution of the binding agent, the impregnated carrier film is dried, preferably at a temperature of from 120 to 215° F. and stored until ready for use. Prior to using the carrier film, it is passed through a humidifying apparatus at a temperature of about 100° F. in an atmosphere of about 90 to 100% relative humidity for such time as is required to impart to the impregnated carrier film a moisture content of from 20 to 40%.

The film is then in a limp condition and should be laid between the sheets to be laminated and subjected to the hot pressing operation as soon as possible thereafter. Either wood veneer or wood fiber board may be used as the constituent lamination in the manufacture of plywood or other laminated product.

Upon the application of heat and pressure in the hot press, the resinous material with which the carrier film is impregnated fuses and is converted into a hard, infusible resin. Due to the fact that the resinous material of the carrier film contains the proper amount of moisture, a certain amount of steam will be formed under the influence of heat and serve as a carrier for the fused resin. As the process takes place under constant pressure, the resin binder is forced into the constituent laminations in a fused state in both directions. Upon the continued application of heat, the fused resin sets into a hard infusible and insoluble compound. If the film does not

contain sufficient moisture, the penetration of the binder into the wood is limited, owing to its dry state, and the resulting bond will be inferior.

In the hot pressing operation best results are obtained by the use of temperatures between 315° and 335° F., and pressures ranging between 100 lbs. and 250 lbs. per sq. in. The time required will, of course, depend upon the temperature and the thickness of the plywood panel being made, but in general will vary between 2½ and 30 minutes.

The hot panels coming from the hydraulic press are immediately taken to humidifying apparatus, where they are piled between racks and weighted to keep them flat. The humidifying apparatus is then operated at a temperature of about 190° F. and at a relative humidity of 80 to 90%, the length of time in the humidifying equipment depending upon the thickness of the plywood panels and the moisture content desired in the panels. In general, it is desirable to impart to the panels a moisture content of between 8 and 12%. With this moisture content the plywood panels will not be subject to much change when exposed to the relative humidities occurring in most localities in which plywood panels are used.

The aqueous dispersion of the binding material may be prepared from various ingredients capable of forming synthetic resins of a hard, infusible character. Examples of suitable synthetic resins are those of the phenolic-aldehyde and urea-aldehyde type, or mixtures of a urea and of a phenol with an aldehyde, or polymer of an aldehyde, as described in my copending application entitled "Method of making plywood", Serial No. 741,745, filed August 27, 1934.

In addition to the examples of aqueous binder solutions given in the aforesaid application, the following will serve to illustrate methods of preparing suitable binder solutions:

#### Example 1

|                                     | Parts by weight |
|-------------------------------------|-----------------|
| 45 Cresylic acid                    | 1000            |
| Formaldehyde (40% aqueous solution) | 1000            |
| Vegetable protein                   | 200             |
| Caustic soda                        | 160             |
| Soya bean oil                       | 10              |
| 50 Triethanolamine                  | 2½              |
| Water                               | 2400            |

The vegetable protein may be a dry extracted soya bean flour, peanut flour, or the like. Such flour is first added to the cresylic acid with constant stirring until a smooth homogeneous mass results. A 38° Bé. solution of caustic soda, containing about 100 parts of caustic soda, is added to the mixture of cresylic acid and soya bean or the vegetable flour. Then the soya bean oil and triethanolamine are added and the mixture agitated until a smooth homogeneous mass results. The mass is then cooled to 60° F., at which temperature the formaldehyde is added and the whole mixture agitated for 5 minutes. The heat of reaction between the various ingredients normally brings the mass up to about 70 to 85° C., where the mass is maintained for about 25 to 35 minutes. Next a cold, 10° Bé. solution of 60 parts of caustic soda in 2400 parts of water is added to the mass. If desired, the solution may be further diluted by the addition of water without causing a precipitation of the partial condensation product and will remain stable for a long period of time without any increase in viscosity.

#### Example 2

|                                     | Parts by weight |
|-------------------------------------|-----------------|
| Cresylic acid                       | 600             |
| Formaldehyde (40% aqueous solution) | 600             |
| Caustic soda                        | 96              |
| Triethanolamine                     | 1.5             |
| Soya bean oil                       | 1.5             |
| Water                               | 1500            |

In making up this second formula, 60 parts of caustic soda are dissolved in order to form a 30° Bé. solution and this solution then added to the cresylic acid and mixed thoroughly therewith. The mixture is allowed to cool to 60° F., at which temperature the soya bean oil and triethanolamine are added. The formaldehyde is next added and the mixture agitated. The heat of reaction between the various ingredients brings the mass up to a temperature of normally from 70 to 90° C. After maintaining the mass at this temperature for about 25 to 35 minutes, the remaining portion of caustic soda, namely 36 parts, dissolved in 1500 parts of water and having a specific gravity of about 10° Bé., is added to the mixture with constant stirring until cold. As before, the solution may be diluted further by the addition of water without causing a precipitation of the partial condensation product. The final mixture is a clear amber colored solution and will remain stable for a long period of time without any increase in viscosity.

An improved binder solution may be prepared in accordance with the following example:

#### Example 3

After the reaction mixture has been prepared, but before its diluting with the additional water, the partial condensation product is precipitated by the addition of acidulated water, with constant stirring, and then allowed to settle. After decanting off the supernatant liquor, the soft resin material remaining is washed by the further addition of water until the mixture shows no acid reaction, after which the resinous mass is dissolved in the caustic soda solution with constant stirring.

By the method of Example 3, all the impurities are removed from the resin, so that when the resin is brought back into solution, the mixture is much lighter in color and holds for a much longer period of time without any increase in viscosity.

In Examples 1 and 2, soya bean flour or peanut flour are incorporated for the purpose of increasing the bonding strength of the synthetic resin resulting from the reaction between cresylic acid and formaldehyde. Other vegetable products rich in protein, cellulose and carbohydrates may be used.

It will be understood that the proportions of the various ingredients in the formulae of Examples 1 and 2 may be varied considerably and other ingredients substituted for those enumerated, as more fully explained in my copending application above referred to. The caustic soda used aids in increasing the solubility of the initial condensation product produced by the reaction between formaldehyde and cresylic acid, or sodium cresylate. The triethanolamine, which may be a commercial mixture of tri-, di- and monoethanolamine, acts as an emulsifying agent to prevent precipitation of the partial condensation product. It is important to note, however, that the final solution of the binder material is a true aqueous solution and not an emulsion or colloidal suspension. The reaction is not carried beyond

the point at which the partial condensation product is still water soluble.

I am aware that numerous details of the process may be varied through a wide range without departing from the principles of this invention, and I, therefore, do not purpose limiting the patent granted hereon otherwise than necessitated by the prior art.

I claim as my invention:

- 10 1. The method of making laminated products, which comprises impregnating a porous flexible fibrous web with an aqueous solution of a resinous partial condensation product, drying the impregnated web, humidifying said impregnated web 15 to impart thereto a moisture content of from 20 to 40%, laying said humidified web between sheets of the material to be laminated and subjecting the assembled sheets and web to sufficient heat and pressure to effect a bond therebetween.
- 20 2. The method of making laminated products, which comprises impregnating a porous flexible fibrous web with an aqueous solution of a partial condensation product of cresylic acid and an aldehyde, drying the impregnated web, humidifying said impregnated web to impart thereto a moisture content of from 20 to 40%, laying said humidified web between sheets of the material to be laminated, subjecting the assembled sheets and web to sufficient heat and pressure to effect a bond therebetween and humidifying the resulting laminated product to impart thereto a moisture content of from 8 to 12%.

3. The method of making plywood, which comprises impregnating an unsized sheet of kraft paper with an aqueous solution of a partial condensation product of cresylic acid and formaldehyde, drying at a temperature of from 120°-215° F. and humidifying the impregnated sheet 15 until the moisture content thereof is between 20 and 40%, interposing said impregnated sheet between wood veneers and subjecting the veneers and sheet to sufficient heat and pressure to convert the partial condensation product into an 20 infusible resin firmly bonding the laminations together.

JAMES V. NEVIN.